

Jan. 17, 1933.

G. P. BARTHOLOMEW

1,894,438

COKING PROCESS

Filed Oct. 20, 1928



Inventor  
George Pomeroy Bartholomew  
By his Attorney Albert M. Austin

## UNITED STATES PATENT OFFICE

GEORGE POMEROY BARTHOLOMEW, OF ESSEX FELLS, NEW JERSEY, ASSIGNOR TO AMERICAN SMELTING & REFINING COMPANY, OF NEW YORK, N. Y., A CORPORATION OF NEW JERSEY

## COKING PROCESS

Application filed October 20, 1928. Serial No. 313,816.

This invention relates to a process for heat treating liquids, and more particularly, to a new and improved process for treating tar for the formation of creosote and coke.

5 When coal tar is heated to a proper temperature, creosote vapors are driven off, leaving a residue of heavier hydrocarbons or pitch. The pitch may be subjected to further heat treatment whereby all of the volatile 10 constituents are removed and the residue is formed into coke.

The present invention provides for the efficient treatment of tar for the production of creosote and coke in one operation. The 15 operation is carried on cyclically and includes subjecting the tar in a finely divided condition to a temperature sufficiently high to drive off the desired percentage of creosote and to initiate coking of the residue. This residue 20 may be further treated at appropriate temperatures to complete the coking operation. The required heat may be obtained during completion of the coking operation and suitably stored for use in treating the next portion 25 of tar. The cycle of operation accordingly comprises treating the tar in a hot chamber to produce creosote vapor and initiate coking of the residue. The coking operation is then completed in the same chamber 30 and the heat derived therefrom is utilized for treating further quantities of tar.

The process is preferably carried out in a chamber having thick refractory walls which are capable of withstanding a comparatively 35 high temperature and of absorbing a considerable amount of heat during the coking operation.

The invention also consists in certain new 40 and original features of construction and combinations of parts hereinafter set forth and claimed.

Although the novel features which are believed to be characteristic of this invention 45 will be particularly pointed out in the claims appended hereto, the invention itself, as to its objects and advantages, the mode of its operation and the manner of its organization may be better understood by referring 50 to the following description taken in connection with the accompanying drawing form-

ing a part thereof, in which the figure is a diagrammatic representation in vertical section of an oven which may be utilized in carrying on this process.

In the following description and in the 55 claims parts will be identified by specific names for convenience, but they are intended to be as generic in their application to similar parts as the art will permit.

The oven which is disclosed in the figure is 60 of conventional design and comprises walls 9 of refractory material which are held in position by any desired means. A thick coating 10 of clay or other heat resisting material is applied over the oven for the purpose of 65 conserving and storing heat. Charging door 13 is provided for removing the resultant coke and for cleaning. The admission of air may be regulated by varying the opening of said door 13 as by fluting with clay in a manner 70 well known in the art. Pipe 14 is located at the upper portion of the oven and is utilized for removing the creosote vapor to suitable condensing mechanism (not shown). A damper or valve 15 may be included in said 75 pipe for controlling the vapor flow. Pipe 16 enters the center of the oven preferably through pipe 14 and terminates in a spray nozzle 17. Pipe 16 may be supported in any 80 desired manner and is utilized for the admission of liquid tar into the chamber.

The oven, as shown, is essentially of the conventional bee-hive coke oven type, particularly adapted for the preparation of metallurgical coke in massive form. Such 85 massive coke, as prepared in this type of oven, has been the standard metallurgical coke since the earliest days of the industry, due to its physical structure and resulting strength, being particularly adapted for use 90 in blast furnaces.

A pitch coke, prepared in the manner to be hereinafter described, in addition to having the desired structure and strength of ordinary metallurgical coke, is characterized by 95 a freedom from gangue or slag-forming constituents, as it is composed essentially of pure carbon.

In carrying on the present process the oven is first heated by any desired means, as for 100

example, by burning a quantity of pitch coke. The heating is continued until the oven reaches a temperature of some 700° C. to 750° C. and large quantities of heat are absorbed and stored in the walls and in the clay covering. After this temperature is reached the oven is entirely closed with the exception of damper 15 in creosote pipe 14. Coal tar is then admitted through pipe 16 and sprayed into the heated space through nozzle 17. The coal tar spray is introduced in a finely divided condition and is immediately heated by the latent heat contained within the furnace and in the walls thereof to a temperature sufficiently high to drive off a large part of the volatile constituents as creosote vapor which is withdrawn through pipe 14 to a suitable condensing apparatus, not shown. The spraying operation is continued until a bed of semi-coke of substantial thickness is formed and the heat absorbed by the tar reduces the temperature of the furnace to, say, approximately 400° C.

The residue remaining after the creosote vapor is driven off is partly coked and falls to the bottom of the chamber. At the end of the spraying or tar charging period, the residue is allowed to stand in the chamber for an additional period of time during which further quantities of vapor are driven off and removed and the coking operation is continued, the temperature of the oven being maintained at approximately 200° C. to 500° C. During this period only a small quantity of heat is being withdrawn from the oven. Hence the total quantity of heat therein and in the heavy refractory walls is sufficient to prevent a substantial lowering of the temperature.

At the end of this second period, the creosote vapor pipe is closed and a small amount of air is admitted through door 13 or by removing a portion of the clay fluting. This air is utilized for supporting combustion within the coking bed and burning a portion of the coke whereby a sufficient quantity of heat is derived to complete the coking of the residue and to again raise the temperature of the oven to some 800° C. to 900° C.

At the end of this coking period the door is opened and the coke removed. The removal of the coke cools the oven to a slight extent and reduces the temperature thereof to some 700° C. to 750° C. at which temperature a further quantity of tar is charged through pipe 16 and another cycle of operation carried out in the manner above set forth.

In a particular example the tar was sprayed for a period of from 8 to 10 hours, the residue was allowed to remain in the closed chamber for some 39 additional hours and the coking operation required a further period of 28 hours.

In accordance with the above described process, the coal tar is treated for the produc-

tion of creosote and coke without intermediate handling and without the use of external fuel. The coke supplies the heat required for driving off the creosote vapor from subsequent charges of tar. When the residue is completely coked it may be removed through the door of the furnace and is in saleable condition without further treatment.

A comparatively high percentage of creosote recovery is obtained by reason of the efficient heat treatment of the tar. By introducing the same in a finely divided condition it is possible to rapidly raise the temperature thereof to the required value and thereby prevent substantial quantities of intermediate products from being formed.

The process has been described as applied to the treatment of coal tar by way of example only. It is understood that other hydrocarbon oils may be similarly treated at appropriate temperatures for driving off the lighter constituents and leaving the heavy residue.

Although certain novel features of the invention have been shown and described and are pointed out in the annexed claims, it will be understood that various omissions, substitutions and changes in the several steps of the process and in its operation may be made by those skilled in the art without departing from the spirit of the invention.

#### What is claimed is:

1. The process for treating coal tar, which comprises introducing said tar in a finely divided condition into a chamber heated to a temperature of from 400° C. to 900° C. whereby the volatile constituents are removed as vapor and the coking of the residue is begun, collecting said residue as a mass in the bottom of said chamber, admitting small quantities of air to said chamber for burning a portion of coke whereby heat is produced for completing the coking of the residue and for again raising the temperature of said chamber to between 700° C. and 900° C., utilizing the walls of said chamber for storing excess heat, removing the coke from said chamber while maintaining the temperature of the chamber at an operative minimum, and distilling volatiles from a further portion of said tar in the chamber by the so-stored heat.

2. The process for treating coal tar, which comprises introducing said tar in a finely divided condition into a chamber heated to a temperature of approximately 700° C. whereby the volatile constituents are removed as vapor and the coking of the residue is begun, collecting said residue as a coherent mass in said chamber, continuing the introduction of tar until the temperature is reduced to approximately 400° C., discontinuing the introduction of tar and maintaining the residue at approximately 400° C. for a further period of time whereby additional quantities of vapor are driven off, admitting

- small quantities of air to said chamber whereby a portion of coke is burned and heat is produced to complete the coking of the residue and to raise the temperature of said chamber
- 5 to approximately 900° C., utilizing the walls of said chamber for storing excess heat thus produced, removing the coke from said chamber while maintaining the temperature of the chamber at an operative minimum, and dis-
- 10 tilling volatiles from a further portion of said tar in the chamber by the so-stored heat.
3. The process for treating coal tar, which comprises introducing said tar in a finely divided condition into a chamber heated to
- 15 a temperature of from 400° C. to 900° C. whereby the volatile constituents are removed as vapor and the coking of the residue is begun, collecting said residue as a coherent mass in said chamber, maintaining a temperature
- 20 of from 200° C. to 500° C. therein for a further period of time whereby additional quantities of vapor are driven off, then admitting small quantities of air to said chamber whereby a portion of the coke is burned and the
- 25 coking of the residue completed, utilizing the heat thus produced for again raising the temperature of said chamber to between 700° C. and 900° C., utilizing the walls of said chamber for storing excess heat, removing
- 30 the coke from said chamber while maintaining the temperature of the chamber at an operative minimum, and distilling the vola-
- 90 tiles from a further portion of said tar in the chamber by the so-stored heat.
- 35 4. The process for treating coal tar, which comprises spraying said tar into a chamber heated to a temperature of from 400° C. to 900° C. whereby the volatile constituents are removed as vapor and the coking of the
- 40 residue is begun, collecting said residue on the bottom of said chamber, continuing the spraying until a homogeneous mass of substantial thickness has been deposited and the temperature falls to approximately 400° C.,
- 45 then admitting small quantities of air to said chamber whereby a portion of coke is burned, utilizing the heat therefrom for completing the coking of the residue and again raising the temperature of said chamber to between
- 50 700° C. and 900° C., utilizing the walls of said chamber for storing excess heat, removing the coke from said chamber while maintaining the temperature of the chamber at an operative minimum, and distilling volatiles
- 55 from a further portion of said tar in the chamber by the so-stored heat.
5. In the treatment of coal tar for the production of coke, the process which comprises spraying said tar into a closed chamber pre-
- 60 heated to a temperature sufficient to effect simultaneous distillation of creosote and other volatiles and initial coking of the residuum, the heat for said simultaneous distillation and initial coking actions being derived from
- 65 heat stored in the walls of said preheated
- 70
- 75
- 80
- 85
- 90
- 95
- 100
- 105
- 110
- 115
- 120
- 125
- 130